

# UNITED STATES PATENT OFFICE.

ANTONIO MEUCCI, OF CLIFTON, NEW YORK.

## IMPROVEMENT IN TREATING PETROLEUM AND OTHER OILS TO PRODUCE A VEHICLE FOR PAINTS AND VARNISHES.

Specification forming part of Letters Patent No. 36,419, dated September 9, 1862.

*To all whom it may concern:*

Be it known that I, ANTONIO MEUCCI, of Clifton, in the county of Richmond and State of New York, have invented a new and Improved Process for Preparing Hydrocarbon Liquids for Paints, &c.; and I do hereby declare that the following is a full, clear, and exact description of the same.

The object of this invention is to render siccative and consistent such hydrocarbon liquids as petroleum and kerosene, so that the same, when mixed with paints, act as thinners and driers, the same as turpentine.

The invention consists in treating petroleum, coal-oil, or other hydrocarbon liquids or oils with hyponitric gas, substantially in the manner hereinafter described, for the purpose of rendering said oils siccative and fit to be used in paints.

It also consists in mixing with petroleum, kerosene, or other oil, after the same has been treated with hyponitric gas, an extract of the cakes obtained in the manufacture of linseed-oil or of farina of linseed, together with a certain quantity of fish oil, for the purpose of giving to said liquids to required consistency for painting purposes.

To enable those skilled in the art to fully understand and use my invention, I will proceed to describe it.

The petroleum or other oil to be treated with hyponitric gas is put in a vessel which communicates by a suitable pipe with a balloon or retort of glass or other suitable material, in which the hyponitric gas is produced. The preparation of the hyponitric gas can be effected by charging said balloon or retort with three (3) parts of nitric acid to one (1) part of starch, and heating it slowly with steam or in any other desirable manner. After the oil has been exposed to the current of hyponitric gas for about two (2) hours it assumes a dark-green or a reddish-yellow color, which indicates that the operation is finished. The oil must now

be repeatedly washed with clean water until all traces of the acid disappear, and after this is accomplished the oil is heated in a suitable vessel or still by means of a steam-coil or in any other desirable manner for the purpose of expelling the water. By this process petroleum, kerosene, or other oils are rendered siccative, and they can now be used with advantage in paints. After I have treated the petroleum or other oils with hyponitric acid, and in order to increase their consistency or "body" I add to each one hundred (100) gallons of said oils about fifty (50) pounds of linseed or from one hundred (100) to one hundred and fifty (150) pounds of linseed "cakes," (obtained in the manufacture of linseed-oil,) and from twenty (20) to twenty-five (25) gallons of fish-oil, heating the mixture to about 150° to 200° Fahrenheit for from six (6) to eight (8) hours, and stirring it well during the whole operation. It is then left to stand, and after a long rest the oil is drawn off and the residue is pressed.

The oil obtained by this process can be used with advantage for paints. It is very cheap, it has a body equal to linseed-oil or nearly so, and it dries in a short time.

Having thus fully described my invention, what I claim as new, and desire to secure by Letters Patent, is—

1. The employment or use of hyponitric acid in treating petroleum, kerosene, or other oils, substantially in the manner and for the purpose described.

2. Mixing petroleum or other oils after they have been exposed to a current of hyponitric acid, as described, with linseed or with linseed cakes and fish-oil, substantially in the manner and about in the proportions herein specified.

ANTONIO MEUCCI.

Witnesses:

R. GAWLEY,  
TIMOTHY SHINE.